

Dec. 18, 1923.

1,477,869

H. P. DONLE

ELECTRONIC EMISSION

Filed Feb. 3, 1923



Harold P. Donle

INVENTOR

By *J. J. Flynn*  
ATTORNEY

## UNITED STATES PATENT OFFICE.

HAROLD POTTER DONLE, OF MERIDEN, CONNECTICUT, ASSIGNOR TO THE CONNECTICUT TELEPHONE AND ELECTRIC COMPANY, INCORPORATED, OF MERIDEN, CONNECTICUT, A CORPORATION OF CONNECTICUT.

## ELECTRONIC EMISSION.

Application filed February 3, 1923. Serial No. 616,660.

To all whom it may concern:

Be it known that I, HAROLD P. DONLE, a citizen of the United States of America, and residing at Meriden, in the county of New Haven and State of Connecticut, have invented new and useful Improvements in Electronic Emission, of which the following is a specification.

The object of my present invention is to increase the operating effectiveness of vacuum tube apparatus having heated electron-emitting cathodes. According to this invention I provide metallic ions within the tube and thus, in addition to furnishing a basis for ionization effects, increase the electron emission of the cathode for a given temperature.

This is a partial continuation of my co-pending application Serial No. 295,897, filed May 9, 1919. I have discovered that metallic ions may conveniently be electrolyzed from the glass wall of the vacuum tube itself. When said tube is made of soda glass, sodium ions are utilized. When a potash glass is used, potassium ions are released.

The increase of filament electron emission referred to above appears to be due to a deposit of such alkali metals upon the cathode itself. It is not difficult to appreciate that if positively charged molecules of sodium or potassium, for instance, are released within the evacuated space of a tube containing anode and cathode, they will be attracted to and deposited upon the cathode. There the electric charge of the ions will necessarily be neutralized and the molecules will constitute a simple metallic coating upon the cathode surface. The effects may be better understood from a consideration of the accompanying drawings where

Figs. 1, 2 and 3 illustrate three stages of a demonstration showing the described increase of electron emission.

Fig. 4 is a graphic illustration of the comparative results under the conditions of Fig. 1 and Fig. 3, and

Fig. 5 shows a tube connected in one of the usual circuits utilized for two-electrode radio receivers.

The vacuum tube 7 shown in Figs. 1, 2, 3 and 5 contains a filamentary cathode 9 and a spiral anode 10. The filament may be of highly refractory metals such as molybdenum, tungsten or tantalum. In Figs. 1, 2

and 3 the neck 8 of the tube is connected to a high vacuum pump (not shown but of any efficient type) for the purpose of maintaining the vacuum during the experiment. In Fig. 5 the neck is shown sealed off after the highest possible evacuation (sufficient to remove as far as possible all traces of residual or occluded gas) has been attained.

The cathode 9 is heated by means of a battery A, whose voltage obviously may be changed for adjustment of cathode temperature. Control of such heating may also be had by means of a resistor in series with the battery A, in the usual way. A second battery B, with potentiometer, is also provided for supplying a controllable potential (measured from the negative terminal of the cathode 9) to the anode 10.

When the cathode 9 is heated to normal temperature, the anode potential of the newly-manufactured tube (represented in Fig. 1) may be varied from say 0 to 40 volts, with connections as shown, and for each anode potential the anode circuit current may be measured by means of ammeter 12. For a particular tube tested in this way it was found that the anode current gradually increased from 0 to 100 microamperes as the potential was increased from 0 to approximately 5 volts, but that this maximum or saturation value of current did not increase with further increments of voltage up to a value as high as 40. It is generally understood that a limitation of current under these conditions is due to a lack of electrons emitted from the cathode, there being only enough electrons in this instance to carry 100 microamperes. In the particular form shown the tube 7 carries in contact with a portion of its outer surface a secondary anode 11. This external electrode may be a band of silver or other metal of like characteristics, applied directly to the outside of the wall of the tube. In Fig. 2 the anode battery B is shown connected to this secondary anode 11, by means of the wire 15, the working anode 10 being left free. The filamentary cathode is heated as before, and the secondary anode potential set at a convenient value.

Under these conditions the heated glass wall of the tube permits the passage of electrons from the cathode through the glass to the external anode, the glass being partly dissociated and, if soda

glass is used, sodium ions thus produced being thrown off into space. These ions are positively charged, hence some necessarily travel to the filamentary cathode and form a coating thereon. A certain amount of sodium travels, either directly or after evaporation from the cathode, to the cooler parts of the tube and forms a bright metallic deposit thereon as indicated at 16; the extent and thickness of this deposit will of course depend upon the sodium content of the glass and the conditions of operation. After the tube is sealed off this deposit will in the heated tube act as a source of sodium for ionization.

Having continued treatment using the connections of Fig. 2 for about five minutes the bright deposit described becomes relatively heavy and practically opaque. If the anode connection 15 is now attached to the working anode 10, as in Fig. 3, another series of measurements of anode current for various voltages may be taken. The tube having been treated as explained, it is found that for a given cathode temperature and anode potential the anode current is much greater. The same tube described in connection with Fig. 1 was so treated, and then remeasured as in Fig. 3; the anode current rose to 2400 microamperes as the potential was increased from 0 to about 24 volts, at which point saturation was reached and the supply of electrons exhausted. The filament temperature being the same as in the first test, it is evident that the emission has been increased some 24-fold by the treatment. The measurements are represented by curves 14 (before treatment) and 17 (after treatment) in Fig. 4.

The vacuum pump connected to the tube at 8 was kept in operation during the three parts of the demonstration illustrated by Figs. 1, 2 and 3, so as to maintain the highest possible vacuum and to remove any gases that might have been present. This operation did not prevent the formation of the metallic deposits described.

I have found that an increase of emission produced in this way is not necessarily permanent. The time the effect will persist depends upon the composition of the glass and the temperature at which the filament is run after treatment, but usually the effect will last for some time before beginning gradually to fall off. However, it is entirely feasible to maintain the condition of maximum emission by maintaining a supply of suitable metallic ions within the tube. This may be done by continuously passing current through the wall of the tube during its periods of operation and thus renewing the deposit upon the cathode by the substantially continuous electrolytic dissociation of the current-carrying glass and the

consequent liberation of sodium, potassium or the like.

The arrangement of Fig. 5 provides one means for maintaining a suitable condition within the tube in this way. The working anode 10 is here provided with a positive potential derived from the battery A by way of a potentiometer 18, and an aerial 19 and telephone receiver 20 are associated with the detector tube in the usual way. The external electrode is supplied with current from battery B through potentiometer 13, as in Fig. 2, and serves to furnish metallic ions while the tube is in operation. The supply of ions for deposition upon the cathode may be augmented by ions produced when electrons from the cathode strike, with sufficient velocity, neutral molecules of the metallic vapor or atmosphere produced within the tube by partial evaporation of the deposits on the filament or walls under the influence of heat.

I have found that the increased emission effect described permits substantial economies in the energy consumed by the filament of a vacuum tube detector, and that the provision of metallic ions permits the use of desirable ionization effects common in vacuum tubes containing residual gas. However, in tubes supplied with metallic ions these effects are stabilized to so great an extent that they may be depended upon to produce uniformly a higher sensitivity than can be secured from the critical and transient ionization phenomena in detector tubes containing residual gas. Moreover, such metallic ionization tubes as I have described may be manufactured in large quantities with practical uniformity, and are not subject to the wide variations which occur in the production of prior art tubes intended to utilize non-metallic gaseous ionization.

It will be noted that the tubes described have an unobstructed path for electrons and ions between the cathode 9 and working anode 10, and consequently that the conduction and other effects taking place in the space between the electrodes are not interfered with or complicated by changes in field intensity or potential gradient which might be introduced by the addition of any interposed electrodes, shields or other obstacles. By the provision of this free electronic and ionic zone the control of the ionization phenomena utilized in my tubes is facilitated.

To maintain the condition giving rise to the effects characterized by increased cathodic emission I may rely in part upon ionization of deposited bodies of sodium, potassium or the like upon the interior wall of the tube. The supply of ions thus secured serves to augment those produced directly by electrolytic dissociation within the tube

walls. The proportion of the total ionization required for this effect from either source may be varied, and I may supplement or add to the internal deposit by introducing 5 a suitable metal or metals during manufacture of the tube. In fact many desirable and novel effects may be produced by introducing sodium, potassium or the like, into the tube instead of relying upon electrolysis during or after exhaustion.

It should be understood that many advantages of metallic ionization as herein set forth may be obtained in tubes having three internal electrodes, such as are described 15 and claimed in my original application Serial No. 295,897 or in my applications Serial Nos. 579,828 and 604,312. The two last named applications disclose structures in which, as in the present case, an unob- 20 structed path is provided for electron and ion flow between anode and cathode.

It is characteristic of the ionization effects utilized by me that they are non-progressive and non-luminous. That is to say, al- 25 though sufficient ionization within the tube is produced within the tube to provide means for increasing filament electron emission, the ionization is not sufficiently violent or intense as to produce light. If the anode 30 voltage applied to one of these tubes is increased beyond the values best for detecting or amplifying effects, it is possible

to secure luminous ionization but under such conditions the tubes are substantially if not wholly useless as detectors or amplifiers. 35

I claim:

1. The method of increasing the electron emission of a filamentary cathode at a given temperature which consists in continuously attracting to said cathode electrically 40 charged particles of sodium.

2. The method of increasing the electron emission of a filamentary cathode at a given temperature which consists in continuously attracting to said cathode electrically 45 charged particles of an alkali metal.

3. In a radio signalling system a vacuum tube having a highly refractory filamentary cathode, and an anode with an unobstructed electron path therebetween, a deposit of an 50 alkali metal within said tube and means for maintaining a coating of alkali metal on said cathode, all in combination with means for impressing radio frequency potentials upon electrodes of said tube and a translating device connected thereto.

4. In a radio signalling system a wave intercepting device, a vacuum tube having an anode and a highly refractory filamentary cathode with a coating of alkali metal, 60 and a translating device operatively connected therewith.

HAROLD POTTER DONLE.